

May 30, 1933.

E. V. COLLINS, JR

1,911,808

METHOD OF COLORING COAL

Filed Nov. 28, 1930



INVENTOR

Ernest Victor Collins Jr.

BY

Perkins, Drinker, Bacon & Elleray  
ATTORNEYS

## UNITED STATES PATENT OFFICE

ERNEST VICTOR COLLINS, JR., OF BROOKLYN, NEW YORK, ASSIGNOR TO DELAWARE,  
LACKAWANNA & WESTERN COAL COMPANY, OF NEW YORK, N. Y., A CORPORATION  
OF NEW JERSEY

## METHOD OF COLORING COAL

Application filed November 28, 1930. Serial No. 498,685.

This invention relates to the application of color to coal, and has for its object the provision of a simple and effective procedure whereby a surface film of color can 5 be applied to coal in an economical manner to give the coal a distinctive characteristic.

In carrying out the invention, I employ suitable chemical reagents which, when combined, will produce a coloring agent 10 which is adapted to adhere to the surface of coal. Among such reagents are mixtures of ferric chloride and alkali ferricyanides, mixtures of ferric nitrate and alkali ferricyanides, mixtures of potassium permanganate and ferric chloride or nitrate. In using 15 solutions containing ferric chloride or nitrate and alkali ferricyanides, I have found it desirable to employ in addition a small quantity of acid, such as sulphuric, hydrochloric or nitric acid in the solution. In solutions 20 of potassium permanganate and ferric chloride or nitrate, it is desirable to add sulphuric or nitric acid. The foregoing reagents are cited merely as examples, and 25 other reagents capable of reacting to produce coloring agents on the surface of the coal may be employed in practicing the invention.

I have discovered that to obtain the most 30 effective results in the application of color to coal, with reagents such as those mentioned, it is desirable to prepare and maintain separate solutions in water of the respective reagents and to combine such solutions approximately at the time of application 35 thereof to the coal. The application of the solutions in this manner avoids premature reaction and loss of some of the coloring agent. It is not essential that the solutions be combined at the instant of application 40 to the coal. The flowing streams of reagent solutions may be brought together and combined to form a single stream which is then directed upon the coal. I 45 prefer, however, to employ a suitable spray nozzle in which the two solutions are combined and by which a spray of the combined solutions is directed upon the coal which is supported, preferably, upon a traveling 50 conveyor which moves the coal beneath

the spray nozzle. The coal may, however, be arranged in stationary layers or piles and the combined solutions may be directed thereon in the form of a spray or otherwise, or the coal may be moved on a traveling 55 conveyor through a bath which is constantly renewed by the introduction of the separate streams of reagents, the bath being preferably of limited volume so that the combined solutions are exhausted substantially as produced, that is to say, no considerable volume 60 of the combined solutions is permitted to stand for any considerable length of time when coal is not being treated therein. Thus I am able to employ the solutions most 65 economically and effectively, avoiding losses due to premature reaction of the reagents.

I find it advantageous, moreover, to connect a source of electrical current respectively to the combined solutions and to the coal 70 through a suitable metallic support upon which the coal is treated. The function of the electrical current is not readily explainable, but I have discovered that the film of color upon the coal is improved through the 75 application of the electrical current in the manner indicated, probably caused by ionization or lowering the surface tension of the solutions on the surfaces of the coal. The nature and other characteristics of the electrical current appear to have little, if any, effect upon the results secured. Polarity is not important, and I may utilize, therefore, either direct or alternating current. The amount of current flowing is, in any case, 80 relatively slight. I have found that as little as one-sixth of a millampere is sufficient to accomplish the purpose of the invention. The voltage likewise seems to be of relatively slight importance, so long as 85 there is sufficient potential to effect a flow of current. I have found, for example, that a potential of 230 volts is sufficient. Lower or higher voltage may be used, depending upon the particular conditions. A convenient 90 arrangement for the application of current to the coal is a connection from one pole of a source of current to a metallic plate or conveyor upon which the coal rests, the other pole being connected to the nozzle 95 100

through which the combined solutions are directed upon the coal.

I believe that the improved results observed in the application of electrical current in the procedure as described depends upon the provision of an electrical charge upon each of the droplets constituting the spray of combined solutions, and that this charge is dissipated when the droplets strike the coal, thus causing the reaction to speed up as well as to spread the solution over the surface of the coal more readily and thoroughly. As hereinbefore indicated, however, I am by no means certain that the explanation indicated is scientifically correct, and I do not wish, therefore, to be bound by any explanation or theory, since the results described have been obtained and observed in the application of reagents to the surface of coal in the manner indicated.

The invention will be more readily understood by reference to the accompanying drawing, which illustrates diagrammatically a type of apparatus adapted for the application of the procedure, it being understood that other and equivalent means may be utilized.

Referring to the drawing, 5 indicates a suitable conveyor, preferably a metallic belt traveling over suitable pulleys or sprockets 6 in the direction indicated by the arrow. The conveyor may be operated from any suitable source of power. A hopper 7 is filled with lumps of coal 8 which are delivered continuously to the conveyor. As the coal travels on the conveyor it is subjected to a spray of combined solutions of chemicals from a spray nozzle 9 which is supplied through pipes 10 and 11 from sources in which quantities of solutions of the reagents are separately maintained. The coal upon which the spray of combined solutions is directed travels with the conveyor and is discharged into a hopper 12 from which it may be withdrawn. In traveling on the conveyor the coal is more or less coated with the combined solutions, which by reaction produce the coloring agent. The film of color may be apparent while the coal is still wet with the solutions, and as the coal dries the film becomes more apparent and imparts to the coal a characteristic appearance. The film is relatively stable, is not easily removed by washing or abrasion, and the colored coal may be marketed, therefore, as a distinct and recognizable product.

As hereinbefore indicated, it is desirable to apply electrical current from a suitable source to the coal undergoing treatment. As indicated in the drawing, a generator 13 or other suitable source of current is provided, and a conductor 14 is connected to one pole of the generator and to the nozzle 9. The other pole is connected by a conductor 15 to the journal 16 of one of the pulleys or

sprockets 6, and thus to the conveyor 5 traveling thereon. With this arrangement current is permitted to flow while the spray of combined solutions is directed upon the coal in any manner and with the object hereinbefore described.

As examples of the procedure, I may prepare solutions containing 5 pounds of ferric chloride crystals to 100 gallons of water, and 6 pounds of an alkali ferricyanide such as potassium ferricyanide to 100 gallons of water, and these solutions separately maintained may be introduced to the spray nozzle 9, mingled therein, and directed upon the coal. I find it desirable to add to one or the other of these solutions approximately 2 pounds of nitric acid per hundred gallons of water. In place of ferric chloride crystals in one of the solutions, I prefer to employ 14 pounds of ferric nitrate per hundred gallons of water, and to add thereto 2 pounds of nitric acid per hundred gallons of water. When the solutions as described are combined and spread upon coal, either with or without the application of electrical current, the reaction results in depositing on the coal an insoluble film of Prussian blue or related chemical compound, which imparts to the coal a distinctive color characteristic. The color is generally bluish, but as the film is relatively thin and tends to be iridescent, it may range from blue to violet and even include orange and yellow.

A similar brownish film may be produced by preparing one per cent solutions of potassium permanganate and of ferric chloride or nitrate with the addition of about one per cent of sulphuric acid to either solution. Such solutions may be maintained separately and combined at approximately the time of application to the coal. The resulting film is an oxide or hydrated oxide of manganese and iron, and when applied to coal imparts thereto an iridescent color effect.

The temperatures at which the solutions are maintained and applied to the coal may be varied widely. The reaction tends to be more rapid as the temperature rises, and it is desirable, therefore, to heat the solutions to a temperature above atmospheric, although satisfactory results can be secured at temperatures above 45 to 50° F. If the solutions are to be heated, steam can be introduced thereto at the spray nozzle or otherwise, or heat can be applied by steam coils immersed in the receptacles for the respective solutions.

The methods described are merely illustrations of different procedures which can be used in carrying out the invention, and the explanations of reactions herein presented are likewise merely for the purpose of illustration and are not intended to limit the invention.

Various changes may be made in the de-

tails of the procedure, the reagents employed therein, and the apparatus utilized without departing from the invention or sacrificing any of the advantages thereof.

5 I claim:

1. The method of coloring coal which comprises establishing separate flowing streams of solutions of chemical reagents which when combined will produce a coloring agent, bringing the streams of solutions together approximately at the time of application thereof, directing a spray of the combined solutions upon the coal to be treated, and connecting a source of electrical current respectively to the coal and to the combined solutions.

2. The method of coloring coal which comprises establishing separate flowing streams of solutions of chemical reagents which when combined will produce a coloring agent, bringing the streams of solutions together approximately at the time of application thereof, directing the solutions as combined upon the coal to be treated, and connecting a source of electrical current respectively to the coal and to the combined solutions.

3. The method of coloring coal which comprises establishing separate flowing streams of solutions of ferric chloride and an alkali ferricyanide, bringing the streams of solutions together approximately at the time of application thereof, and treating the coal with the solutions as combined.

35 4. The method of coloring coal which comprises establishing separate flowing streams of solutions of ferric chloride and an alkali ferricyanide, one of the streams containing also an acid, bringing the streams of solutions together approximately at the time of application thereof, and treating the coal with the solutions as combined.

5. The method of coloring coal which comprises establishing separate flowing streams of solutions of ferric nitrate and an alkali ferricyanide, bringing the streams together approximately at the time of application thereof, and treating the coal with the solutions as combined.

50 6. The methods of coloring coal which comprises establishing separate flowing streams of solutions of ferric nitrate and an alkali ferricyanide, one of the streams containing also an acid, bringing the streams together approximately at the time of application thereof and treating the coal with the solutions as combined.

60 7. The method of coloring coal which comprises establishing separate flowing solutions of ferric chloride and an alkali ferricyanide, bringing the streams of solutions together approximately at the time of application thereof and directing a spray of the combined solutions upon the coal to be treated.

8. The method of coloring coal which comprises establishing separate flowing solutions of ferric chloride and an alkali ferricyanide, one of the streams containing also an acid, bringing the streams of solutions together approximately at the time of application thereof and directly a spray of the combined solutions upon the coal to be treated.

75 9. The method of coloring coal which comprises establishing separate flowing solutions of ferric nitrate and an alkali ferricyanide, bringing the streams of solutions together approximately at the time of application thereof and directing a spray of the combined solutions upon the coal to be treated.

80 10. The method of coloring coal which comprises establishing separate flowing solutions of ferric nitrate and an alkali ferricyanide, one of the streams containing also an acid, bringing the streams of solutions together approximately at the time of application thereof and directing a spray of the combined solutions upon the coal to be treated.

85 11. The method of coloring coal which comprises establishing separate flowing solutions of ferric chloride and an alkali ferricyanide, bringing the streams of solutions together approximately at the time of the application thereof, directing a spray of the combined solutions upon the coal to be treated, and connecting a source of electrical current respectively to the coal and to the combined solutions.

90 12. The method of coloring coal which comprises establishing separate flowing solutions of ferric chloride and an alkali ferricyanide, one of the streams containing also an acid, bringing the streams of solutions together approximately at the time of application thereof, directing a spray of the combined solutions upon the coal to be treated, and connecting a source of electrical current respectively to the coal and to the combined solutions.

95 13. The method of coloring coal which comprises establishing separate flowing solutions of ferric nitrate and an alkali ferricyanide, bringing the streams of solutions together approximately at the time of application thereof, directing a spray of the combined solutions upon the coal to be treated, and connecting a source of electrical current respectively to the coal and to the combined solutions.

100 14. The method of coloring coal which comprises establishing separate flowing solutions of ferric nitrate and an alkali ferricyanide, one of the streams containing also an acid, bringing the streams of solutions together approximately at the time of application thereof, directing a spray of the combined solutions upon the coal to be treated,

and connecting a source of electrical current respectively to the coal and to the combined solutions.

15. The method of depositing a colored metal salt upon coal which comprises establishing a flowing stream of a solution of a compound of the metal, the salt of which it is desired to deposit upon the coal, establishing a separate flowing stream of a solution of a chemical reagent which will react with the flowing stream of the metal compound to produce the colored metal salt, bringing the streams of solutions together approximately at the time of application thereof, and treating the coal with the solutions as combined.
16. The method of depositing a colored metal salt upon coal which comprises establishing a flowing stream of a solution of a compound of the metal, the salt of which it is desired to deposit upon the coal, establishing a separate flowing stream of a solution of a chemical reagent which will react with the flowing stream of the metal compound to produce the colored metal salt, bringing the streams of solutions together approximately at the time of application thereof, and directing the solutions as combined upon the coal to be treated.
17. The method of depositing a colored metal salt upon coal which comprises establishing a flowing stream of a solution of a compound of the metal, the salt of which it is desired to deposit upon the coal, establishing a separate flowing stream of a solution of a chemical reagent which will react with the flowing stream of the metal compound to produce the colored metal salt, bringing the streams of solutions together approximately at the time of application thereof, and directing a spray of the combined solutions upon the coal to be treated.

In testimony whereof I affix my signature.

ERNEST VICTOR COLLINS, JR.